# EUROPEAN PATENT SPECIFICATION

(11) **EP 2 478 140 B1**
(45) Date of publication and mention of the grant of the patent: **13.11.2013**
(21) Application number: 09849611.0
(22) Date of filing: 15.09.2009
(51) Int. Cl.: D04H 3/14, D04H 3/16, A47L 13/17, A47L 13/16

(54) **COFORM NONWOVEN WEB FORMED FROM MELTBLOWN FIBERS INCLUDING PROPYLENE/ALPHA-OLEFIN**
KOFORMES VLIES AUS SCHMELZGEBLASENEN FASERN MIT PROPYLEN/ALPHA-OLEFIN
VOILE NON TISSÉ COMPOSITE FORMÉ À PARTIR DE FIBRES FONDUES-SOUFFLÉES COMPRENANT DU PROPYLÈNE/DES ALPHA-OLÉFINES

(43) Date of publication of application: 25.07.2012
(73) Proprietor: Kimberly-Clark Worldwide, Inc., Neenah, Wisconsin 54957-0349 (US)
(72) Inventor: JACKSON, David, M., Alpharetta GA 30022 (US); SCHMIDT, Michael, A., Alpharetta GA 30022 (US)
(74) Representative: Beacham, Annabel Rose
(86) International application number: PCT/US2009/057041
(87) International publication number: WO 2011/034523

(56) References cited:
- EP-A2- 0 590 307
- WO-A1-2008/073101
- KR-A- 20060 129 240
- KR-A- 20060 130 230
- KR-A- 20070 006 931
- KR-A- 20080 038 230
- KR-A- 20090 014 302
- US-A1- 2002 155 776
- US-A1- 2005 148 261
- US-A1- 2007 049 153

## Description

### Background of the Invention

Coform nonwoven webs, which are composites of a matrix of meltblown fibers and an absorbent material (e.g., pulp fibers), have been used as an absorbent layer in a wide variety of applications, including absorbent articles, absorbent dry wipes, wet wipes, and mops. Most conventional coform webs employ meltblown fibers formed from polypropylene homopolymers. One problem sometimes experienced with such coform materials, however, is that the polypropylene meltblown fibers do not readily bond to the absorbent material. Thus, to ensure that the resulting web is sufficiently strong, a relatively high percentage of meltblown fibers are typically employed to enhance the degree of bonding at the crossover points of the meltblown fibers. Unfortunately, the use of such a high percentage of meltblown fibers may have an adverse affect on the resulting absorbency of the coform web. Another problem sometimes experienced with conventional coform webs relates to the ability to form a textured surface. For example, a textured surface may be formed by contacting the meltblown fibers with a foraminous surface having three-dimensional surface contours. With conventional coform webs, however, it is sometimes difficult to achieve the desired texture due to the relative inability of the meltblown fibers to conform to the three-dimensional contours of the foraminous surface.

As such, a need currently exists for an improved coform nonwoven web for use in a variety of applications.

### Summary of the Invention

In accordance with one embodiment of the present invention, a coform nonwoven web is disclosed that comprises a matrix of meltblown fibers and an absorbent material. The meltblown fibers are formed from a thermoplastic composition that contains at least one propylene/α-olefin copolymer having a propylene content of from 60 mole% to 99.5 mole% and an α-olefin content of from 0.5 mole% to 40 mole%. The copolymer further has a density of from 0.86 to 0.90 grams per cubic centimeter and the thermoplastic composition has melt flow rate of from 200 to 6000 grams per 10 minutes, determined at 230°C in accordance with ASTM Test Method D1238-E.

In accordance with another embodiment of the present invention, a method of forming a coform nonwoven web is disclosed that comprises merging together a stream of an absorbent material with a stream of meltblown fibers to form a composite stream. Thereafter, the composite stream is collected on a forming surface to form a coform nonwoven web. The meltblown fibers are formed from a thermoplastic composition such as described above.

Other features and aspects of the present invention are described in more detail below.

### Brief Description of the Drawings

A full and enabling disclosure of the present invention, including the best mode thereof, directed to one of ordinary skill in the art, is set forth more particularly in the remainder of the specification, which makes reference to the appended figures in which:
Fig. 1 is a schematic illustration one embodiment of a method for forming the coform web of the present invention;
Fig. 2 is an illustration of certain features of the apparatus shown in Fig. 1; and
Fig. 3 is a cross-sectional view of one embodiment of a textured coform nonwoven web formed according to the present invention.

Repeat use of reference characters in the present specification and drawings is intended to represent same or analogous features or elements of the invention.

### Detailed Description of Representative Embodiments Definitions

As used herein the term "nonwoven web" generally refers to a web having a structure of individual fibers or threads which are interlaid, but not in an identifiable manner as in a knitted fabric. Examples of suitable nonwoven fabrics or webs include, but are not limited to, meltblown webs, spunbond webs, bonded carded webs, airlaid webs, coform webs, hydraulically entangled webs, and so forth.

As used herein, the term "meltblown web" generally refers to a nonwoven web that is formed by a process in which a molten thermoplastic material is extruded through a plurality of fine, usually circular, die capillaries as molten fibers into converging high velocity gas (e.g., air) streams that attenuate the fibers of molten thermoplastic material to reduce their diameter, which may be to microfiber diameter. Thereafter, the meltblown fibers are carried by the high velocity gas stream and are deposited on a collecting surface to form a web of randomly dispersed meltblown fibers. Such a process is disclosed, for example, in U.S. Patent No. 3,849,241 to Butin, et al.. Generally speaking, meltblown fibers may be microfibers that are substantially continuous or discontinuous, generally smaller than 10 micrometers in diameter, and generally tacky when deposited onto a collecting surface.

As used herein, the term "spunbond web" generally refers to a web containing small diameter substantially continuous fibers. The fibers are formed by extruding a molten thermoplastic material from a plurality of fine, usually circular, capillaries of a spinnerette with the diameter of the extruded fibers then being rapidly reduced as by, for example, eductive drawing and/or other well-known spunbonding mechanisms. The production of spunbond webs is described and illustrated, for example, in U.S. Patent Nos. 4,340,563 to Appel, et al., 3,692,618 to Dorschner, et al., 3,802,817 to Matsuki, et al., 3,338,992 to Kinney, 3,341,394 to Kinney, 3,502,763 to Hartman, 3,502,538 to Levy, 3,542,615 to Dobo, et al., and 5,382,400 to Pike, et al.. Spunbond fibers are generally not tacky when they are deposited onto a collecting surface. Spunbond fibers may sometimes have diameters less than 40 micrometers, and are often between 5 to 20 micrometers.

### Detailed Description

Reference now will be made in detail to various embodiments of the invention, one or more examples of which are set forth below. Each example is provided by way of explanation, not limitation of the invention. In fact, it will be apparent to those skilled in the art that various modifications and variations may be made in the present invention without departing from the scope or spirit of the invention. For instance, features illustrated or described as part of one embodiment, may be used on another embodiment to yield a still further embodiment. Thus, it is intended that the present invention cover such modifications and variations.

Generally speaking, the present invention is directed to a coform nonwoven web that contains a matrix of meltblown fibers and an absorbent material. The meltblown fibers are formed from a thermoplastic composition that contains at least one propylene/α-olefin copolymer of a certain monomer content, density, melt flow rate, etc. The selection of a specific type of propylene/α-olefin copolymer provides the resulting composition with improved thermal properties for forming a coform web. For example, the thermoplastic composition crystallizes at a relatively slow rate, thereby allowing the fibers to remain slightly tacky during formation. This tackiness may provide a variety of benefits, such as enhancing the ability of the meltblown fibers to adhere to the absorbent material during web formation. Due in part to its enhanced bonding capacity, a lower amount of meltblown fibers may also be employed than previously thought needed to form a coherent and self-supporting coform structure. For example, the meltblown fibers may constitute from 2 wt.% to 40 wt.%, in some embodiments from 4 wt.% to 30 wt.%, and in some embodiments, from 5 wt.% to 20 wt.% of the coform web. Likewise, the absorbent material may constitute from 60 wt.% to 98 wt.%, in some embodiments from 70 wt.% to 96 wt.%, and in some embodiments, from 80 wt.% to 95 wt.% of the coform web.

In addition to enhancing the bonding capacity of the meltblown fibers, the thermoplastic composition of the present invention may also impart other benefits to the resulting coform structure. In certain embodiments, for example, the coform web may be imparted with texture using a three-dimensional forming surface. In such embodiments, the relatively slow rate of crystallization of the meltblown fibers may increase their ability to conform to the contours of the three-dimensional forming surface. Once the fibers crystallize, however, the meltblown fibers may achieve a degree of stiffness similar to conventional polypropylene, thereby allowing them to retain their three-dimensional shape and form a highly textured surface on the coform web.

Another benefit of the fiber's prolonged tackiness during formation may be an increased ply attachment strength between layers of a multi-ply coform nonwoven web, resulting in additional shear energy being necessary to delaminate the plies. Such increased ply attachment strength may reduce or eliminate the need for embossing that could negatively impact sheet characteristics such as thickness and density. Increased ply attachment strength may be particularly desirable during dispensing of wipers made from a multi-ply coform nonwoven web. Texture imparted by using a three-dimensional forming surface as described herein may further increase the ply attachment strength by increasing the contact surface area between the plies.

Various embodiments of the present invention will now be described in more detail.

### I Thermoplastic Composition

The thermoplastic composition of the present invention contains at least one copolymer of propylene and an α-olefin, such as a C₂-C₂₀ α-olefin, C₂-C₁₂ α-olefin, or C₂-C₈ α-olefin. Suitable α-olefins may be linear or branched (e.g., one or more C₁-C₃ alkyl branches, or an aryl group). Specific examples include ethylene, butene; 3-methyl-1-butene; 3,3-dimethyl-1-butene; pentene; pentene with one or more methyl, ethyl or propyl substituents; hexene with one or more methyl, ethyl or propyl substituents; heptene with one or more methyl, ethyl or propyl substituents; octene with one or more methyl, ethyl or propyl substituents; nonene with one or more methyl, ethyl or propyl substituents; ethyl, methyl or dimethyl-substituted decene; dodecene; styrene; and so forth. Particularly desired α-olefin comonomers are ethylene, butene (e.g., 1-butene), hexene, and octene (e.g., 1-octene or 2-octene). The propylene content of such copolymers may be from 60 mole% to 99.5 mole%, in some embodiments from 80 mole% to 99 mole%, and in some embodiments, from 85 mole% to 98 mole%. The α-olefin content may likewise range from 0.5 mole% to 40 mole%, in some embodiments from 1 % to 20 mole%, and in some embodiments, from 2 mole% to 15 mole%. The distribution of the α-olefin comonomer is typically random and uniform among the differing molecular weight fractions forming the propylene copolymer.

The density of the propylene/α-olefin copolymer may be a function of both the length and amount of the α-olefin. That is, the greater the length of the α-olefin and the greater the amount of α-olefin present, the lower the density of the copolymer. Generally speaking, copolymers with a higher density are better able to retain a three-dimensional structure, while those with a lower density possess better elastomeric properties. Thus, to achieve an optimum balance between texture and stretchability, the propylene/α-olefin copolymer is normally selected to have a density of 0.86 grams per cubic centimeter (g/cm³) to 0.90 g/cm³, in some embodiments from 0.861 to 0.89 g/cm³, and in some embodiments, from 0.862 g/cm³ to 0.88 g/cm³. Further, the density of the thermoplastic composition is normally selected to have a density of 0.86 grams per cubic centimeter (g/cm³) to 0.94 g/cm³, in further embodiments from 0.861 to 0.92 g/cm³, and in even further embodiments, from 0.862 g/cm³ to 0.90 g/cm³.

Any of a variety of known techniques may generally be employed to form the propylene/α-olefin copolymer used in the meltblown fibers. For instance, olefin polymers may be formed using a free radical or a coordination catalyst (e.g., Ziegler-Natta). Preferably, the copolymer is formed from a single-site coordination catalyst, such as a metallocene catalyst. Such a catalyst system produces propylene copolymers in which the comonomer is randomly distributed within a molecular chain and uniformly distributed across the different molecular weight fractions. Metallocene-catalyzed propylene copolymers are described, for instance, in U.S. Patent Nos. 7,105,609 to Datta, et al.; 6,500,563 to Datta, et al.; 5,539,056 to Yang, et al.; and 5,596,052 to Resconi, et al.. Examples of metallocene catalysts include bis(n-butylcyclopentadienyl)titanium dichloride, bis(n-butylcyclopentadienyl)zirconium dichloride, bis(cyclopentadienyl)scandium chloride, bis(indenyl)zirconium dichloride, bis(methylcyclopentadienyl)titanium dichloride, bis(methylcyclopentadienyl)zirconium dichloride, cobaltocene, cyclopentadienyltitanium trichloride, ferrocene, hafnocene dichloride, isopropyl(cyclopentadienyl,-1-flourenyl)zirconium dichloride, molybdocene dichloride, nickelocene, niobocene dichloride, ruthenocene, titanocene dichloride, zirconocene chloride hydride, zirconocene dichloride, and so forth. Polymers made using metallocene catalysts typically have a narrow molecular weight range. For instance, metallocene-catalyzed polymers may have polydispersity numbers (M_{w}/Mₙ) of below 4, controlled short chain branching distribution, and controlled isotacticity.

In particular embodiments the propylene/α-olefin copolymer constitutes 50 wt.% or more, in further embodiments from 60 wt.% or more, and in even further embodiments, 75 wt.% or more of the thermoplastic composition used to form the meltblown fibers. In other embodiments the propylene/α-olefin copolymer constitutes at least 1 wt.% and less than 49 wt.%, in particular embodiments from at least 1% and less than 45 wt.%, in further embodiments from at least 5% and less than 45 wt.%, and in even further embodiments, from at least 5 wt.% and less than 35 wt.% of the thermoplastic composition used to form the meltblown fibers. Of course other thermoplastic polymers may also be used to form the meltblown fibers so long as they do not adversely affect the desired properties of the composite. For example, the meltblown fibers may contain other polyolefins (e.g., polypropylene, polyethylene, etc.), polyesters, polyurethanes, polyamides, block copolymers, and so forth. In one embodiment, the meltblown fibers may contain an additional propylene polymer, such as homopolypropylene or a copolymer of propylene. The additional propylene polymer may, for instance, be formed from a substantially isotactic polypropylene homopolymer or a copolymer containing equal to or less than 10 weight percent of other monomer, i.e., at least 90% by weight propylene. Such a polypropylene may be present in the form of a graft, random, or block copolymer and may be predominantly crystalline in that it has a sharp melting point above 110°C, in some embodiments above 115°C, and in some embodiments, above 130°C. Examples of such additional polypropylenes are described in U.S. Patent No. 6,992,159 to Datta, et al..

In particular embodiments, additional polymer(s) may constitute from 0.1 wt.% to 50 wt.%, in further embodiments from 0.5 wt.% to 40 wt.%, and in even further embodiments, from 1 wt.% to 30 wt.% of the thermoplastic composition. Likewise, the above-described propylene/α-olefin copolymer may constitute from 50 wt.% to 99.9 wt.%, in further embodiments from 60 wt.% to 99.5 wt.%, and in even further embodiments, from 75 wt.% to 99 wt.% of the thermoplastic composition.

In other embodiments, additional polymer(s) may constitute from greater than 50wt%, in particular embodiments from 50 wt% to 99 wt%, in selected embodiments from 55 wt% to 99 wt%, in further embodiments from 55 wt.% to 95 wt.%, and in even further embodiments from 65 wt % to 95 wt%. Likewise, the above described propylene/α-olefin copolymer may constitute from less than 49 wt %, in particular embodiments from 1 wt.% to 49 wt.%, in selected embodiments from 1 wt.% to 45 wt.%, in further embodiments from 5 wt.% to 45 wt.%, and in even further embodiments, from 5 wt.% to 35 wt.% of the thermoplastic composition.

The thermoplastic composition used to form the meltblown fibers may also contain other additives as is known in the art, such as melt stabilizers, processing stabilizers, heat stabilizers, light stabilizers, antioxidants, heat aging stabilizers, whitening agents, etc. Phosphite stabilizers (e.g., IRGAFOS available from Ciba Specialty Chemicals of Terrytown, New York and DOVERPHOS available from Dover Chemical Corp. of Dover, Ohio) are exemplary melt stabilizers. In addition, hindered amine stabilizers (e.g., CHIMASSORB available from Ciba Specialty Chemicals) are exemplary heat and light stabilizers. Further, hindered phenols are commonly used as an antioxidant. Some suitable hindered phenols include those available from Ciba Specialty Chemicals of under the trade name "Irganox®", such as Irganox® 1076, 1010, or E 201. When employed, such additives (e.g., antioxidant, stabilizer, etc.) may each be present in an amount from 0.001 wt.% to 15 wt.%, in some embodiments, from 0.005 wt.% to 10 wt.%, and in some embodiments, 0.01 wt.% to 5 wt.% of the thermoplastic composition used to form the meltblown fibers.

Through the selection of certain polymers and their content, the resulting thermoplastic composition may possess thermal properties superior to polypropylene homopolymers conventionally employed in meltblown webs. For example, the thermoplastic composition is generally more amorphous in nature than polypropylene homopolymers conventionally employed in meltblown webs. For this reason, the rate of crystallization of the thermoplastic composition is slower, as measured by its "crystallization half-time" - i.e., the time required for one-half of the material to become crystalline. For example, the thermoplastic composition typically has a crystallization half-time of greater than 5 minutes, in some embodiments from 5.25 minutes to 20 minutes, and in some embodiments, from 5.5 minutes to 12 minutes, determined at a temperature of 125°C. To the contrary, conventional polypropylene homopolymers often have a crystallization half-time of 5 minutes or less. Further, the thermoplastic composition may have a melting temperature ("Tₘ") of from 100°C to 250°C, in some embodiments from 110°C to 200°C, and in some embodiments, from 140°C to 180°C. The thermoplastic composition may also have a crystallization temperature ("T_{c}") (determined at a cooling rate of 10°C/min) of from 50°C to 150°C, in some embodiments from 80°C to 140°C, and in some embodiments, from 100°C to 120°C. The crystallization half-time, melting temperature, and crystallization temperature may be determined using differential scanning calorimetry ("DSC") as is well known to those skilled in the art and described in more detail below.

The melt flow rate of the thermoplastic composition may also be selected within a certain range to optimize the properties of the resulting meltblown fibers. The melt flow rate is the weight of a polymer (in grams) that may be forced through an extrusion rheometer orifice (0.0825-inch diameter) (2.1 mm) when subjected to a force of 2160 grams in 10 minutes at 230°C. Generally speaking, the melt flow rate is high enough to improve melt processability, but not so high as to adversely interfere with the binding properties of the fibers to the absorbent material. Thus, in most embodiments of the present invention, the thermoplastic composition has a melt flow rate of from 120 to 6000 grams per 10 minutes, in some embodiments from 150 to 3000 grams per 10 minutes, and in some embodiments, from 170 to 1500 grams per 10 minutes, measured in accordance with ASTM Test Method D1238-E.

### II. Meltblown Fibers

The meltblown fibers may be monocomponent or multicomponent. Monocomponent fibers are generally formed from a polymer or blend of polymers extruded from a single extruder. Multicomponent fibers are generally formed from two or more polymers (e.g., bicomponent fibers) extruded from separate extruders. The polymers may be arranged in substantially constantly positioned distinct zones across the cross-section of the fibers. The components may be arranged in any desired configuration, such as sheath-core, side-by-side, pie, island-in-the-sea, three island, bull's eye, or various other arrangements known in the art. Various methods for forming multicomponent fibers are described in U.S. Patent Nos. 4,789,592 to Taniguchi et al. and U.S. Patent No. 5,336,552 to Strack et al., 5,108,820 to Kaneko, et al., 4,795,668 to Kruege, et al., 5,382,400 to Pike, et al., 5,336,552 to Strack, et al., and 6,200,669 to Marmon, et al.. Multicomponent fibers having various irregular shapes may also be formed, such as described in U.S. Patent Nos. 5,277,976 to Hogle, et al., 5,162,074 to Hills, 5,466,410 to Hills, 5,069,970 to Largman, et al., and 5,057,368 to Largman, et al..

### III. Absorbent Material

Any absorbent material may generally be employed in the coform nonwoven web, such as absorbent fibers, particles, etc. In one embodiment, the absorbent material includes fibers formed by a variety of pulping processes, such as kraft pulp, sulfite pulp, thermomechanical pulp, etc. The pulp fibers may include softwood fibers having an average fiber length of greater than 1 mm and particularly from 2 to 5 mm based on a length-weighted average. Such softwood fibers can include, but are not limited to, northern softwood, southern softwood, redwood, red cedar, hemlock, pine (e.g., southern pines), spruce (e.g., black spruce), combinations thereof, and so forth. Exemplary commercially available pulp fibers suitable for the present invention include those available from Weyerhaeuser Co. of Federal Way, Washington under the designation "Weyco CF-405 " Hardwood fibers, such as eucalyptus, maple, birch, aspen, and so forth, can also be used. In certain instances, eucalyptus fibers may be particularly desired to increase the softness of the web. Eucalyptus fibers can also enhance the brightness, increase the opacity, and change the pore structure of the web to increase its wicking ability. Moreover, if desired, secondary fibers obtained from recycled materials may be used, such as fiber pulp from sources such as, for example, newsprint, reclaimed paperboard, and office waste. Further, other natural fibers can also be used in the present invention, such as abaca, sabai grass, milkweed floss, pineapple leaf, and so forth. In addition, in some instances, synthetic fibers can also be utilized.

Besides or in conjunction with pulp fibers, the absorbent material may also include a superabsorbent that is in the form fibers, particles, gels, etc. Generally speaking, superabsorbents are water-swellable materials capable of absorbing at least 20 times its weight and, in some cases, at least 30 times its weight in an aqueous solution containing 0.9 weight percent sodium chloride. The superabsorbent may be formed from natural, synthetic and modified natural polymers and materials. Examples of synthetic superabsorbent polymers include the alkali metal and ammonium salts of poly(acrylic acid) and poly(methacrylic acid), poly(acrylamides), poly(vinyl ethers), maleic anhydride copolymers with vinyl ethers and alpha-olefins, poly(vinyl pyrrolidone), poly(vinylmorpholinone), poly(vinyl alcohol), and mixtures and copolymers thereof. Further, superabsorbents include natural and modified natural polymers, such as hydrolyzed acrylonitrile-grafted starch, acrylic acid grafted starch, methyl cellulose, chitosan, carboxymethyl cellulose, hydroxypropyl cellulose, and the natural gums, such as alginates, xanthan gum, locust bean gum and so forth. Mixtures of natural and wholly or partially synthetic superabsorbent polymers may also be useful in the present invention. Particularly suitable superabsorbent polymers are HYSORB 8800AD (BASF of Charlotte, North Carolina and FAVOR SXM 9300 (available from Degussa Superabsorber of Greensboro, North Carolina).

### IV. Coform Technique

The coform web of the present invention is generally made by a process in which at least one meltblown die head (e.g., two) is arranged near a chute through which the absorbent material is added while the web forms. Some examples of such coform techniques are disclosed in U.S. Patent Nos. 4,100,324 to Anderson, et al., 5,350,624 to Georger, et al., and 5,508,102 to Georger, et al., as well as U.S. Patent Application Publication Nos. 2003/0200991 to Keck, et al. and 2007/0049153 to Dunbar, et al..

Referring to Fig. 1, for example, one embodiment of an apparatus is shown for forming a coform web of the present invention. In this embodiment, the apparatus includes a pellet hopper 12 or 12' of an extruder 14 or 14', respectively, into which a propylene/α-olefin thermoplastic composition may be introduced. The extruders 14 and 14' each have an extrusion screw (not shown), which is driven by a conventional drive motor (not shown). As the polymer advances through the extruders 14 and 14', it is progressively heated to a molten state due to rotation of the extrusion screw by the drive motor. Heating may be accomplished in a plurality of discrete steps with its temperature being gradually elevated as it advances through discrete heating zones of the extruders 14 and 14' toward two meltblowing dies 16 and 18, respectively. The meltblowing dies 16 and 18 may be yet another heating zone where the temperature of the thermoplastic resin is maintained at an elevated level for extrusion.

When two or more meltblowing die heads are used, such as described above, it should be understood that the fibers produced from the individual die heads may be different types of fibers. That is, one or more of the size, shape, or polymeric composition may differ, and furthermore the fibers may be monocomponent or multicomponent fibers. For example, larger fibers may be produced by the first meltblowing die head, such as those having an average diameter of 10 micrometers or more, in some embodiments 15 micrometers or more, and in some embodiments, from 20 to 50 micrometers, while smaller fibers may be produced by the second die head, such as those having an average diameter of 10 micrometers or less, in some embodiments 7 micrometers or less, and in some embodiments, from 2 to 6 micrometers. In addition, it may be desirable that each die head extrude approximately the same amount of polymer such that the relative percentage of the basis weight of the coform nonwoven web material resulting from each meltblowing die head is substantially the same. Alternatively, it may also be desirable to have the relative basis weight production skewed, such that one die head or the other is responsible for the majority of the coform web in terms of basis weight. As a specific example, for a meltblown fibrous nonwoven web material having a basis weight of 1.0 ounces per square yard or "osy" (34 grams per square meter or "gsm"), it may be desirable for the first meltblowing die head to produce 30 percent of the basis weight of the meltblown fibrous nonwoven web material, while one or more subsequent meltblowing die heads produce the remainder 70 percent of the basis weight of the meltblown fibrous nonwoven web material. Generally speaking, the overall basis weight of the coform nonwoven web is from 10 gsm to 350 gsm, and more particularly from 17 gsm to 200 gsm, and still more particularly from 25 gsm to 150 gsm.

Each meltblowing die 16 and 18 is configured so that two streams of attenuating gas per die converge to form a single stream of gas which entrains and attenuates molten threads 20 and 21 as they exit small holes or orifices 24 in each meltblowing die. The molten threads 20 and 21 are formed into fibers or, depending upon the degree of attenuation, microfibers, of a small diameter which is usually less than the diameter of the orifices 24. Thus, each meltblowing die 16 and 18 has a corresponding single stream of gas 26 and 28 containing entrained thermoplastic polymer fibers. The gas streams 26 and 28 containing polymer fibers are aligned to converge at an impingement zone 30. Typically, the meltblowing die heads 16 and 18 are arranged at a certain angle with respect to the forming surface, such as described in U.S. Patent Nos. 5,508,102 and 5,350,624 to Georger et al. Referring to Fig. 2, for example, the meltblown dies 16 and 18 may be oriented at an angle α as measured from a plane "A" tangent to the two dies 16 and 18. As shown, the plane "A" is generally parallel to the forming surface 58 (Fig. 1). Typically, each die 16 and 18 is set at an angle ranging from 30 to 75 degrees, in some embodiments from 35° to 60°, and in some embodiments from 45° to 55°. The dies 16 and 18 may be oriented at the same or different angles. In fact, the texture of the coform web may actually be enhanced by orienting one die at an angle different than another die.

Referring again to Fig. 1, absorbent fibers 32 (e.g., pulp fibers) are added to the two streams 26 and 28 of thermoplastic polymer fibers 20 and 21, respectively, and at the impingement zone 30. Introduction of the absorbent fibers 32 into the two streams 26 and 28 of thermoplastic polymer fibers 20 and 21, respectively, is designed to produce a graduated distribution of absorbent fibers 32 within the combined streams 26 and 28 of thermoplastic polymer fibers. This may be accomplished by merging a secondary gas stream 34 containing the absorbent fibers 32 between the two streams 26 and 28 of thermoplastic polymer fibers 20 and 21 so that all three gas streams converge in a controlled manner. Because they remain relatively tacky and semi-molten after formation, the meltblown fibers 20 and 21 may simultaneously adhere and entangle with the absorbent fibers 32 upon contact therewith to form a coherent nonwoven structure.

To accomplish the merger of the fibers, any conventional equipment may be employed, such as a picker roll 36 arrangement having a plurality of teeth 38 adapted to separate a mat or batt 40 of absorbent fibers into the individual absorbent fibers. When employed, the sheets or mats 40 of fibers 32 are fed to the picker roll 36 by a roller arrangement 42. After the teeth 38 of the picker roll 36 have separated the mat of fibers into separate absorbent fibers 32, the individual fibers are conveyed toward the stream of thermoplastic polymer fibers through a nozzle 44. A housing 46 encloses the picker roll 36 and provides a passageway or gap 48 between the housing 46 and the surface of the teeth 38 of the picker roll 36. A gas, for example, air, is supplied to the passageway or gap 46 between the surface of the picker roll 36 and the housing 48 by way of a gas duct 50. The gas duct 50 may enter the passageway or gap 46 at the junction 52 of the nozzle 44 and the gap 48. The gas is supplied in sufficient quantity to serve as a medium for conveying the absorbent fibers 32 through the nozzle 44. The gas supplied from the duct 50 also serves as an aid in removing the absorbent fibers 32 from the teeth 38 of the picker roll 36. The gas may be supplied by any conventional arrangement such as, for example, an air blower (not shown). It is contemplated that additives and/or other materials may be added to or entrained in the gas stream to treat the absorbent fibers. The individual absorbent fibers 32 are typically conveyed through the nozzle 44 at about the velocity at which the absorbent fibers 32 leave the teeth 38 of the picker roll 36. In other words, the absorbent fibers 32, upon leaving the teeth 38 of the picker roll 36 and entering the nozzle 44, generally maintain their velocity in both magnitude and direction from the point where they left the teeth 38 of the picker roll 36. Such an arrangement, which is discussed in more detail in U.S. Patent No. 4,100,324 to Anderson, et al.

If desired, the velocity of the secondary gas stream 34 may be adjusted to achieve coform structures of different properties. For example, when the velocity of the secondary gas stream is adjusted so that it is greater than the velocity of each stream 26 and 28 of thermoplastic polymer fibers 20 and 21 upon contact at the impingement zone 30, the absorbent fibers 32 are incorporated in the coform nonwoven web in a gradient structure. That is, the absorbent fibers 32 have a higher concentration between the outer surfaces of the coform nonwoven web than at the outer surfaces. On the other hand, when the velocity of the secondary gas stream 34 is less than the velocity of each stream 26 and 28 of thermoplastic polymer fibers 20 and 21 upon contact at the impingement zone 30, the absorbent fibers 32 are incorporated in the coform nonwoven web in a substantially homogenous fashion. That is, the concentration of the absorbent fibers is substantially the same throughout the coform nonwoven web. This is because the low-speed stream of absorbent fibers is drawn into a high-speed stream of thermoplastic polymer fibers to enhance turbulent mixing which results in a consistent distribution of the absorbent fibers.

To convert the composite stream 56 of thermoplastic polymer fibers 20, 21 and absorbent fibers 32 into a coform nonwoven structure 54, a collecting device is located in the path of the composite stream 56. The collecting device may be a forming surface 58 (e.g., belt, drum, wire, fabric, etc.) driven by rollers 60 and that is rotating as indicated by the arrow 62 in Fig. 1. The merged streams of thermoplastic polymer fibers and absorbent fibers are collected as a coherent matrix of fibers on the surface of the forming surface 58 to form the coform nonwoven web 54. If desired, a vacuum box (not shown) may be employed to assist in drawing the near molten meltblown fibers onto the forming surface 58. The resulting textured coform structure 54 is coherent and may be removed from the forming surface 58 as a self-supporting nonwoven material.

It should be understood that the present invention is by no means limited to the above-described embodiments. In an alternative embodiment, for example, first and second meltblowing die heads may be employed that extend substantially across a forming surface in a direction that is substantially transverse to the direction of movement of the forming surface. The die heads may likewise be arranged in a substantially vertical disposition, i.e., perpendicular to the forming surface so that the thus-produced meltblown fibers are blown directly down onto the forming surface. Such a configuration is well known in the art and described in more detail in, for instance, U.S. Patent Application Publication No. 2007/0049153 to Dunbar, et al. Furthermore, although the above-described embodiments employ multiple meltblowing die heads to produce fibers of differing sizes, a single die head may also be employed. An example of such a process is described, for instance, in U.S. Patent Application Publication No. 2005/0136781 to Lassig, et al..

As indicated above, it is desired in certain cases to form a coform web that is textured. Referring again to Fig. 1, for example, one embodiment of the present invention employs a forming surface 58 that is foraminous in nature so that the fibers may be drawn through the openings of the surface and form dimensional cloth-like tufts projecting from the surfaces of the material that correspond to the openings in the forming surface 58. The foraminous surface may be provided by any material that provides sufficient openings for penetration by some of the fibers, such as a highly permeable forming wire. Wire weave geometry and processing conditions may be used to alter the texture or tufts of the material. The particular choice will depend on the desired peak size, shape, depth, surface tuft "density" (that is, the number of peaks or tufts per unit area), etc. In one embodiment, for example, the wire may have an open area of from about 35% and about 65%, in some embodiments from about 40% to about 60%, and in some embodiments, from about 45% to about 55%. One exemplary high open area forming surface is the forming wire FORMTECH™ 6 manufactured by Albany International Co. of Albany, New York. Such a wire has a "mesh count" of about six strands by six strands per square inch (about 2.4 by 2.4 strands per square centimeter), i.e., resulting in about 36 foramina or "holes" per square inch (about 5.6 per square centimeter), and therefore capable of forming about 36 tufts or peaks in the material per square inch (about 5.6 peaks per square centimeter). The FORMTECH™ 6 wire also has a warp diameter of about 1 millimeter polyester, a shute diameter of about 1.07 millimeters polyester, a nominal air permeability of approximately 41.8 m³/min (1475 ft³/min), a nominal caliper of about 0.2 centimeters (0.08 inch) and an open area of approximately 51%. Another exemplary forming surface available from the Albany International Co. is the forming wire FORMTECH™ 10, which has a mesh count of about 10 strands by 10 strands per square inch (about 4 by 4 strands per square centimeter), i.e., resulting in about 100 foramina or "holes" per square inch (about 15.5 per square centimeter), and therefore capable of forming about 100 tufts or peaks per square inch (about 15.5 peaks per square centimeter) in the material. Still another suitable forming wire is FORMTECH™ 8, which has an open area of 47% and is also available from Albany International. Of course, other forming wires and surfaces (e.g., drums, plates, etc.) may be employed. Also, surface variations may include but are not limited to, alternate weave patterns, alternate strand dimensions, release coatings (e.g., silicones, fluorochemicals, etc.), static dissipation treatments, and the like. Still other suitable foraminous surfaces that may be employed are described in U.S. Patent Application Publication No. 2007/0049153 to Dunbar, et al.

Regardless of the particular texturing method employed, the tufts formed by the meltblown fibers of the present invention are better able to retain the desired shape and surface contour. Namely, because the meltblown fibers crystallize at a relatively slow rate, they are soft upon deposition onto the forming surface, which allows them to drape over and conform to the contours of the surface. After the fibers crystallize, they are then able to hold the shape and form tufts. The size and shape of the resulting tufts depends upon the type of forming surface used, the types of fibers deposited thereon, the volume of below wire air vacuum used to draw the fibers onto and into the forming surface, and other related factors. For example, the tufts may project from the surface of the material in the range of 0.25 millimeters to at least 5 millimeters, and in some embodiments, from 0.5 millimeters to 3 millimeters. Generally speaking, the tufts are filled with fibers and thus have desirable resiliency useful for wiping and scrubbing.

Fig. 3 shows an illustration of a cross section of a textured coform web 100 having a first exterior surface 122 and a second exterior surface 128. At least one of the exterior surfaces has a three-dimensional surface texture. In Fig. 3, for instance, the first exterior surface 122 has a three-dimensional surface texture that includes tufts or peaks 124 extending upwardly from the plane of the coform material One indication of the magnitude of three-dimensionality in the textured exterior surface(s) of the coform web is the peak to valley ratio, which is calculated as the ratio of the overall thickness "T" divided by the valley depth "D." When textured in accordance with the present invention, the coform web typically has a peak to valley ratio of 5 or less, in some embodiments from 0.1 to 4 and in some embodiments, from 0.5 to 3. The number and arrangement of the tufts 24 may vary widely depending on the desired end use. In particular embodiments, the textured coform web will have from 2 and 70 tufts per square centimeter, and in other embodiments, from 5 and 50 tufts per square centimeter. In certain embodiments, the textured coform web will have from 100 to 20,000 tufts per square meter, and in further embodiments will have from 200 to 10,000 tufts per square meter. The textured coform web may also exhibit a three-dimensional texture on the second surface of the web. This will especially be the case for lower basis weight materials, such as those having a basis weight of less than 70 grams per square meter due to "mirroring", wherein the second surface of the material exhibits peaks offset or between peaks on the first exterior surface of the material. In this case, the valley depth D is measured for both exterior surfaces as above and are then added together to determine an overall material valley depth.

### V. Articles

The coform nonwoven web may be used in a wide variety of articles. For example, the web may be incorporated into an "absorbent article" that is capable of absorbing water or other fluids. Examples of some absorbent articles include, but are not limited to, personal care absorbent articles, such as diapers, training pants, absorbent underpants, incontinence articles, feminine hygiene products (e.g., sanitary napkins), swim wear, baby wipes, mitt wipe, and so forth; medical absorbent articles, such as garments, fenestration materials, underpads, bedpads, bandages, absorbent drapes, and medical wipes; food service wipers; clothing articles; pouches, and so forth. Materials and processes suitable for forming such articles are well known to those skilled in the art.

In one particular embodiment of the present invention, the coform web is used to form a wipe. The wipe may be formed entirely from the coform web or it may contain other materials, such as films, nonwoven webs (e.g., spunbond webs, meltblown webs, carded web materials, other coform webs, airlaid webs, etc.), paper products, and so forth. In one embodiment, for example, two layers of a textured coform web may be laminated together to form the wipe, such as described in U.S. Patent Application Publication No. 2007/0065643 to Kopacz. In such embodiments, one or both of the layers may be formed from the coform web of the present invention. In another embodiment, it may be desired to provide a certain amount of separation between a user's hands and a moistening or saturating liquid that has been applied to the wipe, or, where the wipe is provided as a dry wiper, to provide separation between the user's hands and a liquid spill that is being cleaned up by the user. In such cases, an additional nonwoven web or film may be laminated a surface of the coform web to provide physical separation and/or provide liquid barrier properties. Other fibrous webs may also be included to increase absorbent capacity, either for the purposes of absorbing larger liquid spills, or for the purpose of providing a wipe a greater liquid capacity. When employed, such additional materials may be attached to the coform web using any method known to one skilled in the art, such as by thermal or adhesive lamination or bonding with the individual materials placed in face to face contacting relation. Regardless of the materials or processes utilized to form the wipe, the basis weight of the wipe is typically from 20 to 200 grams per square meter (gsm), and in some embodiments, between 35 to 100 gsm. Lower basis weight products may be particularly well suited for use as light duty wipes, while higher basis weight products may be better adapted for use as industrial wipes.

The wipe may assume a variety of shapes, including but not limited to, generally circular, oval, square, rectangular, or irregularly shaped. Each individual wipe may be arranged in a folded configuration and stacked one on top of the other to provide a stack of wet wipes. Such folded configurations are well known to those skilled in the art and include c-folded, z-folded, quarter-folded configurations and so forth. For example, the wipe may have an unfolded length of from 2.0 to 80.0 centimeters, and in some embodiments, from 10.0 to 25.0 centimeters. The wipes may likewise have an unfolded width of from 2.0 to 80.0 centimeters, and in some embodiments, from 10.0 to 25.0 centimeters. The stack of folded wipes may be placed in the interior of a container, such as a plastic tub, to provide a package of wipes for eventual sale to the consumer. Alternatively, the wipes may include a continuous strip of material which has perforations between each wipe and which may be arranged in a stack or wound into a roll for dispensing. Various suitable dispensers, containers, and systems for delivering wipes are described in U.S. Patent Nos. 5,785,179 to Buczwinski, et al.; 5,964,351 to Zander; 6,030,331 to Zander; 6,158,614 to Haynes, et al.; 6,269,969 to Huang, et al.; 6,269,970 to Huang, et al.; and 6,273,359 to Newman, et al..

In certain embodiments of the present invention, the wipe is a "wet" or "premoistened" wipe in that it contains a liquid solution for cleaning, disinfecting, sanitizing, etc. The particular liquid solutions are not critical and are described in more detail in U.S. Patent Nos. 6,440,437 to Krzysik, et al.; 6,028,018 to Amundson, et al.; 5,888,524 to Cole; 5,667,635 to Win, et al.; and 5,540,332 to Kopacz, et al.. The amount of the liquid solution employed may depending upon the type of wipe material utilized, the type of container used to store the wipes, the nature of the cleaning formulation, and the desired end use of the wipes. Generally, each wipe contains from 150 to 600 wt.% and desirably from 300 to 500 wt.% of a liquid solution based on the dry weight of the wipe.

The present invention may be better understood with reference to the following examples.

### Test Methods

### Melt Flow Rate:

The melt flow rate ("MFR") is the weight of a polymer (in grams) forced through an extrusion rheometer orifice (0.0825-inch diameter) (2.1 mm) when subjected to a load of 2160 grams in 10 minutes at 230°C. Unless otherwise indicated, the melt flow rate was measured in accordance with ASTM Test Method D1238-E.

### Thermal Properties:

The melting temperature, crystallization temperature, and crystallization half time were determined by differential scanning calorimetry (DSC) in accordance with ASTM D-3417. The differential scanning calorimeter was a DSC Q100 Differential Scanning Calorimeter, which was outfitted with a liquid nitrogen cooling accessory and with a UNIVERSAL ANALYSIS 2000 (version 4.6.6) analysis software program, both of which are available from T.A. Instruments Inc. of New Castle, Delaware. To avoid directly handling the samples, tweezers or other tools were used. The samples were placed into an aluminum pan and weighed to an accuracy of 0.01 milligram on an analytical balance. A lid was crimped over the material sample onto the pan. Typically, the resin pellets were placed directly in the weighing pan, and the fibers were cut to accommodate placement on the weighing pan and covering by the lid.

The differential scanning calorimeter was calibrated using an indium metal standard and a baseline correction was performed, as described in the operating manual for the differential scanning calorimeter. A material sample was placed into the test chamber of the differential scanning calorimeter for testing, and an empty pan is used as a reference. All testing was run with a 55-cubic centimeter per minute nitrogen (industrial grade) purge on the test chamber. For resin pellet samples, the heating and cooling program was a 2-cycle test that began with an equilibration of the chamber to -25°C, followed by a first heating period at a heating rate of 10°C per minute to a temperature of 200°C, followed by equilibration of the sample at 200°C for 3 minutes, followed by a first cooling period at a cooling rate of 10°C per minute to a temperature of -25°C, followed by equilibration of the sample at -25°C for 3 minutes, and then a second heating period at a heating rate of 10°C per minute to a temperature of 200°C. All testing was run with a 55-cubic centimeter per minute nitrogen (industrial grade) purge on the test chamber. The results were then evaluated using the UNIVERSAL ANALYSIS 2000 analysis software program, which identified and quantified the melting and crystallization temperatures.

The half time of crystallization was separately determined by melting the sample at 200°C for 5 minutes, quenching the sample from the melt as rapidly as possible in the DSC to a preset temperature, maintaining the sample at that temperature, and allowing the sample to crystallize isothermally. Tests were performed at two different temperatures - i.e., 125°C and 130°C. For each set of tests, heat generation was measured as a function of time while the sample crystallized. The area under the peak was measured and the time which divides the peak into two equal areas was defined as the half-time of crystallization. In other words, the area under the peak was measured and divided into two equal areas along the time scale. The elapsed time corresponding to the time at which half the area of the peak was reached was defined as the half-time of crystallization. The shorter the time, the faster the crystallization rate at a given crystallization temperature.

### EXAMPLE 1

Various grades of polypropylene were tested for their half crystallization time (t_{1/2}) at 125°C and 130°C, crystallization temperature (T_{c}), and melting temperature (Tₘ) as described above. The results are shown below.

| Designation | t_{1/2}[min] @ 125C | t_{1/2}[min] @ 130C | T_{c} [°C] | Tₘ [°C] |
|---|---|---|---|---|
| Basell 441¹ | 2.5 | 9.5 | 111 | 167 |
| Metocene MF650X² | 5.0 | 17.0 | 113 | 156 |
| Borflow HL512³ | 1.3 | 4.0 | 119 | 160 |
| VM 7001-3⁴ | 6.0 | 20.0 | 111 | 158 |

| | | | | |
|---|---|---|---|---|
| ¹ Basell 441 is a propylene homopolymer having a density of 0.91 g/cm³ and melt flow rate of 440 g/10 minute (230°C, 2.16 kg), which is available from Basell Polyolefins. ² Metocene MF650X is a propylene homopolymer having a density of 0.91 g/cm³ and melt flow rate of 1200 g/10 minute (230°C, 2.16 kg), which is available from Basell Polyolefins. ³ Borflow HL512 is a propylene homopolymer having a density of 0.91 g/cm³ and melt flow rate of 1200 g/10 minute (230°C, 2.16 kg), which is available from Borealis A/S. ⁴ [VM 7001-3] is a blend of 75 wt.% propylene homopolymer (Achieve 6936G1) and 25 wt.% propylene/ethylene copolymer (Vistamaxx 2370, density 0.868 g/cm³, meltflow rate of 200 g/10 minutes (230°C, 2.16 kg)) having a density of 0.89 g/cm³ and a melt flow rate of 540 g/10 minutes (230°C, 2.16 kg), which is available from ExxonMobil Corp. | | | | |

### EXAMPLE 2

Various samples of coform webs were formed from two heated streams of meltblown fibers and a single stream of fiberized pulp fibers as described above and shown in Fig. 1. The meltblown fibers were formed from the polypropylene samples referenced in Example 1. The pulp fibers were fully treated southern softwood pulp obtained from the Weyerhaeuser Co. of Federal Way, Washington under the designation "CF-405."

The polypropylene of each stream was supplied to respective meltblown dies at a rate of 1.5 to 2.5 pounds of polymer per inch (0.68 to 1.13 kg per 2.54 cm) of die tip per hour to achieve a meltblown fiber content ranging from 25 wt.% to 40 wt.%. The distance from the impingement zone to the forming wire (i.e., the forming height) was approximately 8 inches (20.3 cm) and the distance between the tips of the meltblown dies was approximately (12.7 cm) 5 inches (12.7 cm). The meltblown die positioned upstream from the pulp fiber stream was oriented at an angle of 50° relative to the pulp stream, while the other meltblown die (positioned downstream from the pulp stream) was oriented between 42 to 45° relative to the pulp stream. The forming wire was FORMTECH™ 8 (Albany International Co.). To achieve different types of tufts, rubber mats were disposed on the upper surface of the forming wire. One such mat had a thickness of approximately 0.95 centimeters and contained holes arranged in a hexagonal array. The holes had a diameter of approximately 0.64 centimeters and were spaced apart approximately 0.95 centimeters (center-to-center). Mats of other patterns (e.g., clouds) were also used. A vacuum box was positioned below the forming wire to aid in deposition of the web and was set to 30 inches of water (7470 Pa).

## Claims

1. A coform nonwoven web comprising a matrix of meltblown fibers and an absorbent material, the meltblown fibers being formed from a thermoplastic composition that contains at least one propylene/α-olefin copolymer having a propylene content of from 60 mole% to 99.5 mole% and an α-olefin content of from 0.5 mole% to 40 mole%, wherein the copolymer further has a density of from 0.86 to 0.90 grams per cubic centimeter and the composition has a melt flow rate of from 120 to 6000 grams per 10 minutes, determined at 230°C in accordance with ASTM Test Method D1238-E.

2. The coform nonwoven web of claim 1, wherein the α-olefin includes ethylene.

3. The coform nonwoven web of claim 1 or 2, wherein propylene constitutes from 85 mole% to 98 mole% of the copolymer and the α-olefin constitutes from 2 mole% to 15 mole% of the copolymer.

4. The coform nonwoven web of any of the foregoing claims, wherein the copolymer has a density of from 0.861 to 0.89 grams per cubic centimeter, and preferably from 0.862 to 0.88 grams per cubic centimeter, and/or wherein the thermoplastic composition has a density from 0.86 to 0.94 grams per cubic centimeter, preferably from 0.861 to 0.92 grams per cubic centimeter, and more preferably from 0.862 to 0.90 grams per cubic centimeter.

5. The coform nonwoven web of any of the foregoing claims, wherein the propylene copolymer is single-site catalyzed.

6. The coform nonwoven web of any of the foregoing claims, wherein the melt flow rate of the composition is from 170 to 1500 grams per 10 minutes.

7. The coform nonwoven web of any of the foregoing claims, wherein the thermoplastic composition has a crystallization half-time of greater than about 5 minutes, and preferably from 5.5 to 12 minutes, measured at 125°C in accordance with ASTM D-3417.

8. The coform nonwoven web of any of the foregoing claims, wherein the propylene/α-olefin copolymer constitutes at least 50 wt.% of the thermoplastic composition, and preferably at least 75 wt.% of the thermoplastic composition.

9. The coform nonwoven web of any one of claims 1 - 7, wherein the propylene/α-olefin copolymer constitutes at least about 1 wt.% and less than 49 wt.% of the thermoplastic composition; preferably wherein the propylene/α-olefin copolymer constitutes at least 5 wt.% and/or less than 45 wt.% of the thermoplastic composition; and more preferably wherein the propylene/α-olefin copolymer constitutes less than 35 wt. % of the thermoplastic composition.

10. The coform nonwoven web of any of the foregoing claims, wherein the absorbent material contains pulp fibers.

11. The coform nonwoven web of any of the foregoing claims, wherein the meltblown fibers constitute from 1 wt.% to 40 wt.% of the web and the absorbent material constitutes from 60 wt.% to 99 wt.% of the web; preferably wherein the meltblown fibers constitute from 5 wt.% to 20 wt.% of the web and the absorbent material constitutes from 80 wt.% to 95 wt.% of the web.

12. The coform nonwoven web of any of the foregoing claims, wherein the web defines an exterior surface having a three-dimensional texture that includes a plurality of peaks and valleys.

13. A wipe comprising the coform nonwoven web of any of the foregoing claims; preferably wherein the wipe contains from 150 to 600 wt.% of a liquid solution based on the dry weight of the wipe.

14. A method of forming a coform nonwoven web as defined in any of claims 1 to 13, the method comprising:
merging together a stream of an absorbent material with a stream of meltblown fibers to form a composite stream, the meltblown fibers being formed from a thermoplastic composition as defined in any of claims 1 to 13; and
thereafter, collecting the composite stream on a forming surface to form a coform nonwoven web.

15. The method of claim 14, wherein the stream of absorbent material is merged together with first and second streams of meltblown fibers; preferably wherein the first stream and second stream of meltblown fibers are supplied from respective first and second die heads, each of which is oriented at an angle of from 45° to 55° relative to a plane tangent to the die heads.

## Patentansprüche

1. Coform-Vliesbahn, welche eine Matrix aus Schmelzblasfasern und ein absorptionsfähiges Material umfasst, wobei die Schmelzblasfasern aus einer thermoplastischen Zusammensetzung gebildet sind, die mindestens ein Propylen/α-Olefin-Copolymer mit einem Propylengehalt von 60 Mol-% bis 99,5 Mol-% und einen α-Olefin-Gehalt von 0,5 Mol-% bis 40 Mol-% enthält, wobei das Copolymer des Weiteren eine Dichte von 0,86 bis 0,90 Gramm pro Kubikzentimeter aufweist und wobei die Zusammensetzung eine Schmelzflussrate von 120 bis 6000 Gramm pro 10 Minuten aufweist, bestimmt bei 230°C in Übereinstimmung mit dem ASTM Testverfahren D1238-E.

2. Coform-Vliesbahn gemäß Anspruch 1, wobei das α-Olefin Ethylen beinhaltet.

3. Coform-Vliesbahn gemäß Anspruch 1 oder 2, wobei Propylen von 85 Mol-% bis 98 Mol-% des Copolymers ausmacht und das α-Olefin 2 Mol-% bis 15 Mol-% des Copolymers ausmacht.

4. Coform-Vliesbahn gemäß einem der vorherigen Ansprüche, wobei das Copolymer eine Dichte von 0,861 bis 0,89 Gramm pro Kubikzentimeter aufweist, und vorzugsweise von 0,862 bis 0,88 Gramm pro Kubikzentimeter, und/oder wobei die thermoplastische Zusammensetzung eine Dichte von 0,86 bis 0,94 Gramm pro Kubikzentimeter aufweist, vorzugsweise von 0,861 bis 0,92 Gramm pro Kubikzentimeter, und noch mehr bevorzugt von 0,862 bis 0,90 Gramm pro Kubikzentimeter.

5. Coform-Vliesbahn gemäß einem der vorherigen Ansprüche, wobei das Propylen-Copolymer einzelstellen-katalysiert ist.

6. Coform-Vliesbahn gemäß einem der vorherigen Ansprüche, wobei die Schmelzflussrate der Zusammensetzung von 170 bis 1500 Gramm pro 10 Minuten beträgt.

7. Coform-Vliesbahn gemäß einem der vorherigen Ansprüche, wobei die thermoplastische Zusammensetzung eine Kristallisationshalbzeit von mehr als ungefähr 5 Minuten aufweist, und vorzugsweise von 5,5 bis 12 Minuten, gemessen bei 125°C in Übereinstimmung mit dem ASTM D-3417.

8. Coform-Vliesbahn gemäß einem der vorherigen Ansprüche, wobei das Propylen/α-Olefin-Copolymer mindestens 50 Gew.-% der thermoplastischen Zusammensetzung ausmacht, und vorzugsweise mindestens 75 Gew.-% der thermoplastischen Zusammensetzung.

9. Coform-Vliesbahn gemäß einem der Ansprüche 1-7, wobei das Propylen/α-Olefin-Copolymer mindestens ungefähr 1 Gew.-% und weniger als 49 Gew.-% der thermoplastischen Zusammensetzung ausmacht, wobei das Propylen/α-Olefin-Copolymer vorzugsweise mindestens 5 Gew.-% und/oder weniger als 45 Gew.-% der thermoplastischen Zusammensetzung ausmacht, und wobei noch mehr bevorzugt das Propylen/α-Olefin-Copolymer weniger als 35 Gew.-% der thermoplastischen Zusammensetzung ausmacht.

10. Coform-Vliesbahn gemäß einem der vorherigen Ansprüche, wobei das absorptionsfähige Material Pulpefasern enthält.

11. Coform-Vliesbahn gemäß einem der vorherigen Ansprüche, wobei die Schmelzblasfasern von 1 Gew.-% bis 40 Gew.-% der Bahn ausmachen und das absorptionsfähige Material von 60 Gew.-% bis 99 Gew.-% der Bahn ausmacht, wobei vorzugsweise die Schmelzblasfasern von 5 Gew.-% bis 20 Gew.-% der Bahn ausmachen und das absorptionsfähige Material von 80 Gew.-% bis 95 Gew.-% der Bahn ausmacht.

12. Coform-Vliesbahn gemäß einem der vorherigen Ansprüche, wobei die Bahn eine Außenoberfläche bestimmt, die eine dreidimensionale Textur aufweist, die eine Vielzahl von Erhebungen und Vertiefungen aufweist.

13. Wischtuch, welches die Coform-Vliesbahn gemäß einem der vorherigen Ansprüche umfasst, wobei das Wischtuch vorzugsweise basierend auf dem Trockengewicht des Wischtuchs 150 bis 600 Gew.-% einer flüssigen Lösung enthält.

14. Verfahren zum Bilden einer Coform-Vliesbahn gemäß einem der Ansprüche 1 bis 13, wobei das Verfahren umfasst:
Zusammenvereinen eines Stroms eines absorptionsfähigen Material mit einem Strom von Schmelzblasfasern, um einen Verbundstoffstrom zu bilden, wobei die Schmelzblasfasern aus einer thermoplastischen Zusammensetzung gemäß einem der Ansprüche 1 bis 13 gebildet sind; und
danach Sammeln des Verbundstoffstroms auf einer Formoberfläche, um eine Coform-Vliesbahn zu bilden.

15. Verfahren gemäß Anspruch 14, wobei der Strom von absorptionsfähigen Material mit einem ersten und zweiten Strom von Schmelzblasfasern vereint wird, wobei vorzugsweise der erste Strom und der zweite Strom von Schmelzblasfasern über entsprechende erste und zweite Düsenköpfe bereitgestellt werden, von welchen jeder mit einem Winkel von 45° bis 55° relativ zu einer Ebene tangential zu den Düsenköpfen ausgerichtet ist.

## Revendications

1. Voile non tissé de co-forme comprenant une matrice de fibres extrudées-soufflées et une matière absorbante, les fibres extrudées-soufflées étant formées à partir d'une composition thermoplastique qui contient au moins un copolymère de propylène/α-oléfine ayant une teneur en propylène de 60 % en mole à 99,5 % en mole et une teneur en α-oléfine de 0,5 % en mole à 40 % en mole, dans lequel le copolymère a en outre une densité de 0,86 à 0, 90 gramme par centimètre cube et la composition a une vitesse d'écoulement à l'état fondu de 120 à 6 000 grammes par 10 minutes, déterminée à 230 °C conformément à la méthode d'essai ASTM D1238-E.

2. Voile non tissé de co-forme selon la revendication 1, dans lequel l'α-oléfine inclut de l'éthylène.

3. Voile non tissé de co-forme selon la revendication 1 ou 2, dans lequel le propylène constitue de 85 % en mole à 98 % en mole du copolymère et l'α-oléfine constitue de 2 % en mole à 15 % en mole du copolymère.

4. Voile non tissé de co-forme selon l'une quelconque des revendications précédentes, dans lequel le copolymère a une densité de 0,861 à 0,89 gramme par centimètre cube, et de préférence de 0,862 à 0,88 gramme par centimètre cube, et/ou dans lequel la composition thermoplastique a une densité de 0,86 à 0,94 gramme par centimètre cube, de préférence de 0,861 à 0,92 gramme par centimètre cube, et de manière plus préférée de 0,862 à 0,90 gramme par centimètre cube.

5. Voile non tissé de co-forme selon l'une quelconque des revendications précédentes, dans lequel le copolymère de propylène est catalysé sur un site unique.

6. Voile non tissé de co-forme selon l'une quelconque des revendications précédentes, dans lequel la vitesse d'écoulement à l'état fondu de la composition est de 170 à 1 500 grammes par 10 minutes.

7. Voile non tissé de co-forme selon l'une quelconque des revendications précédentes, dans lequel la composition thermoplastique a une demi-vie de cristallisation supérieure à environ 5 minutes, et de préférence de 5,5 à 12 minutes, mesurée à 125 °C conformément à l'ASTM D-3417.

8. Voile non tissé de co-forme selon l'une quelconque des revendications précédentes, dans lequel le copolymère de propylène/α-oléfine constitue au moins 50 % en poids de la composition thermoplastique, et de préférence au moins 75 % en poids de la composition thermoplastique.

9. Voile non tissé de co-forme selon l'une quelconque des revendications 1 à 7, dans lequel le copolymère de propylène/α-oléfine constitue au moins environ 1 % en poids et moins de 49 % en poids de la composition thermoplastique ; de préférence dans lequel le copolymère de propylène/α-oléfine constitue au moins 5 % en poids et/ou moins de 45 % en poids de la composition thermoplastique ; et de manière plus préférée dans lequel le copolymère de propylène/α-oléfine constitue moins de 35 % en poids de la composition thermoplastique.

10. Voile non tissé de co-forme selon l'une quelconque des revendications précédentes, dans lequel la matière absorbante contient des fibres de pâte.

11. Voile non tissé de co-forme selon l'une quelconque des revendications précédentes, dans lequel les fibres extrudées-soufflées constituent de 1 % en poids à 40 % en poids du voile et la matière absorbante constitue de 60 % en poids à 99 % en poids du voile ; de préférence dans lequel les fibres extrudées-soufflées constituent de 5 % en poids à 20 % en poids du voile et la matière absorbante constitue de 80 % en poids à 95 % en poids du voile.

12. Voile non tissé de co-forme selon l'une quelconque des revendications précédentes, dans lequel le voile définit une surface extérieure ayant une texture tridimensionnelle qui inclut une pluralité de pics et de vallées.

13. Lingette comprenant le voile non tissé de co-forme selon l'une quelconque des revendications précédentes ; de préférence dans lequel la lingette contient de 150 à 600 % en poids d'une solution liquide sur la base du poids à sec de la lingette.

14. Procédé de formation d'un voile non tissé de co-forme tel que défini dans l'une quelconque des revendications 1 à 13, le procédé comprenant :
réunir ensemble un flux d'une matière absorbante avec un flux de fibres extrudées-soufflées pour former un flux composite, les fibres extrudées-soufflées étant formées à partir d'une composition thermoplastique telle que définie dans l'une quelconque des revendications 1 à 13 ; et
ensuite, recueillir le flux composite sur une surface de formation pour former un voile non tissé de co-forme.

15. Procédé selon la revendication 14, dans lequel le flux de matière absorbante est réuni avec des premier et second flux de fibres extrudées-soufflées ; de préférence dans lequel le premier flux et le second flux de fibres extrudées-soufflées sont fournis à partir de première et seconde têtes de filière respectives, dont chacune est orientée à un angle de 45° à 55° par rapport à un plan tangent aux têtes de filière.
